

## UNITED STATES PATENT OFFICE

1,949,929

## DISSOLVING CADMIUM METAL IN SULPHURIC ACID IN THE PRESENCE OF METALLIC IRON

Harry P. Corson, Lakewood, Ohio, assignor to  
The Grasselli Chemical Company, Cleveland,  
Ohio, a corporation of Delaware

No Drawing. Application November 8, 1932,  
Serial No. 641,761

1 Claim. (Cl. 23—117)

The present invention relates to a process of dissolving metallic cadmium in hot, dilute sulphuric acid and is characterized by the fact that the operation is carried out in the presence of 5 metallic iron.

It is well known that ordinary commercial slabs of metallic cadmium or even feathered cadmium metal dissolve extremely slowly in hot, dilute sulphuric acid, as a matter of fact, I found for 10 instance that only 6% of cadmium metal was dissolved when feathered cadmium was boiled for 48 hours in an excess of 20% sulphuric acid.

I have found that if metallic iron is present in the reaction mixture of sulphuric acid and 15 cadmium metal the rate of attack of the cadmium is considerably accelerated, whereas the iron is only dissolved to a small extent.

The following is an example of how I have operated my novel process:

20 I have, for instance, heated cadmium metal in boiling 20% sulphuric acid in which has been immersed a piece of sheet steel and found that in

48 hours 90 parts of cadmium metal were dissolved whereas only 6 parts of the iron had gone into solution.

Strange enough, I found also that iron salts, such as ferrous sulphate or other metals, such 60 as copper, when present in the sulphuric acid do not materially affect the rate of attack of the sulphuric acid upon the cadmium metal.

The cadmium sulphate solution obtained according to my novel process contains small 65 amounts of ferrous sulphate. This, however, can be removed from the cadmium sulphate solution by well known means. This purification step does not counterbalance the great saving effected 70 by the increased rate of attack by the presence of metallic iron in the reaction mixture.

I claim:

The process of dissolving cadmium metal which comprises boiling metallic cadmium and iron in 75 dilute sulfuric acid solution.

HARRY P. CORSON.

25

80

30

85

35

90

40

95

45

100

50

105

55

110